

A. B. NEWMAN.  
PROCESS OF ROASTING ORES.  
APPLICATION FILED MAR. 23, 1916.

1,280,283.

Patented Oct. 1, 1918.

*Fig. 2.*



*Fig. 1.*



*Inventor:*  
Albert B. Newman

# UNITED STATES PATENT OFFICE.

ALBERT B. NEWMAN, OF LANGELOTH, PENNSYLVANIA, ASSIGNOR TO METALLURGICAL COMPANY OF AMERICA, OF NEW YORK, N. Y., A CORPORATION OF NEW JERSEY.

## PROCESS OF ROASTING ORES.

1,280,283.

Specification of Letters Patent.

Patented Oct. 1, 1918.

Application filed March 23, 1918. Serial No. 86,050.

*To all whom it may concern:*

Be it known that I, ALBERT B. NEWMAN, a citizen of the United States, residing at Langeloth, county of Washington, State of Pennsylvania, have invented certain new and useful Improvements in Processes of Roasting Ores; and I do hereby declare the following to be a full, clear, and exact description of the invention, such as will enable others skilled in the art to which it appertains to make and use the same.

This invention relates to a method of roasting ores, and particularly for roasting zinc sulfid ores and concentrates.

15 The smelting of zinc calcines requires that a minimum of sulfur be retained in them. In order to complete the roasting operation, and effect what is commonly known as a dead roast, extraneous heat is required, particularly near the end of the roasting operation for the purpose of removing the combined sulfur which is not previously removed.

20 Where the sulfur dioxid resulting from the roasting operation is to be used later for the manufacture of sulfuric acid it is desirable that a suitable percentage of sulfur dioxid should be present. This consideration precludes the use of the ordinary heating flames directly in contact with the charge because of the dilution of the roaster gases 30 which would thus take place.

According to the present invention, part or all of the heat necessary to be supplied for effecting and completing the dead roast 35 is supplied by the combustion of sulfur either directly in contact with the charge or indirectly, and the sulfur dioxid formed from the combustion of the sulfur is combined with the roaster gases and the sulfur dioxid content thereof thus further increased. A particularly valuable operation and embodiment of the invention relates to the direct heating of the ore by the combustion of sulfur in direct contact with the 40 charge, whereby the ore is subjected to the heat of combustion of the burning sulfur and the heat necessary for the completion of the roast partially or entirely supplied in this manner.

45 The sulfur can be either in the lump form or in the form of powder, or it can be vola-

tilized and used as a vapor, together with the air necessary to burn it either all at once or in successive stages during its progress through the furnace. The sulfur may thus 55 be burned progressively in the furnace and the heat thereof made available in a progressive manner. Where the sulfur is used in a solid form it can be supplied at different ore hearths and burned with the necessary 60 amount of air so that the resulting products of combustion pass into heating relation to the ore in the ore hearths and so that the sulfur dioxid formed by the combustion of the sulfur combines with the roaster gases 65 and increases their sulfur dioxid content. Where the sulfur is introduced as a vapor it may be all introduced at the lower levels of a multiple hearth furnace and burned all at once or progressively by the introduction of 70 air progressively at different parts of the furnace. The ore in the lower part of the furnace is always hot enough to keep the sulfur volatilized so that the vapor will be carried along with the products of combustion and subsequently burned by the introduction of further amounts of air. It is thus possible to develop heat from the burning sulfur in the lower levels of a multiple hearth furnace where it is most needed to 75 drive off the last part of the combined sulfur from the charge. Instead of supplying heat directly to the ore bed by the combustion of the sulfur in the ore hearths, the heat may be to a greater or less extent supplied by the 80 combustion of sulfur in separate heating flues, in a manner similar to that now commonly practised with producer gas as the heating gas in the heating flues. When sulfur is thus used, however, the sulfur dioxid 85 resulting from its combustion is combined with the roaster gases, as by introducing the sulfur dioxid into the ore hearths, and the roaster gases are thus enriched in sulfur dioxid much the same as when the sulfur is 90 burned in direct contact with the ore bed. So also, where heat is supplied by the combustion of the sulfur in the ore hearths, additional or supplemental amounts of heat can be supplied by burning producer gas or other 95 fuel gas in separate heating flues in much the usual manner without dilution of the roaster 100

2  
gases with the products of combustion of the heating flues. The heat supplied by the combustion of the sulfur in the ore hearths makes it necessary to supply much less heat 5 in the heating flues, with resulting increased efficiency of the roasting operation because of the large loss of heat incident to the indirect heating which must take place through the wall of the gas flue. Accordingly, while 10 the heating with sulfur, either directly or indirectly, is to be considered as within the more general aspects and purposes of the invention, the combustion of the sulfur in the ore hearths and the direct heating of the 15 charge in this manner is a particularly valuable and important embodiment of the invention, whether or not this heating is supplemented by the combustion of added amounts of sulfur or of producer gas or 20 other fuel gas in separate heating flues.

Where the heat is in part or in whole supplied by the combustion of sulfur, either directly or indirectly, and the sulfur dioxid resulting from the combustion of the sulfur 25 is combined with the roaster gases, these gases are enriched in sulfur dioxid and made much richer than gases from the usual roasting operation, with the result that a greater production of acid can be effected therefrom 30 with the same equipment.

In the accompanying drawings, Figure 1 shows, in transverse vertical section, part of a multiple hearth roasting furnace adapted for the practice of the invention, and Fig. 2 shows, in longitudinal vertical section, a modified construction of roasting furnace adapted for the practice of the invention.

Fig. 1 shows half of a double multiple hearth roasting furnace, with the upper portion of the furnace cut away. It will be understood that the other half is of similar construction, as is common in the art, and that a plurality of upper ore hearths will be provided. The inner wall which also 40 forms the inner wall of the other half of the furnace, is indicated at 2. At the lower levels of the furnace are arranged two gas flues 3 and 4 for the combustion therein of producer gas or other combustion gas. 45 These flues communicate with each other by a suitable flue (not shown) in the wall 1 of the furnace similar to the flue 14 of Fig. 2, and a suitable chimney or flue (not shown) is also provided for the escape of the gases 50 from the upper hearth 4. The lower ore hearth 5 is arranged above the gas flue 3 so that it will be heated thereby, and the next ore hearth 6 is arranged to be similarly heated by the gas flue 4, the other upper 55 ore hearths 6 not being heated otherwise than by the heat of the roasting operation.

Opposite the lower hearth 5, and communicating therewith by a suitable flue 8, is a small furnace 7 provided with a bell 60 hopper 10 for the introduction of the sulfur

9 therein and with a suitable regulable air inlet 11. This small furnace will usually be placed near the ore discharge end of the flue 5.

In the usual roasting operation, the heat 70 necessary for completing the roast is furnished by the combustion of producer gas or like fuel gas in the gas flues 3 and 4 which alternate with the lower ore hearths 5 and 6. According to the present invention, where 75 the combustion of sulfur supplies to a greater or less extent the heat necessary for the completion of the roast, the sulfur may be burned in the gas flues 3 and 4, and the resulting sulfur dioxid then utilized for 80 the purpose of enriching the roaster gases.

Where the sulfur is burned in the ore hearths and the heat thereby supplied directly to the charge, less heat is necessary from the heating flues. In order that the 85 heat of the sulfur burned in the ore hearths may be more uniformly applied, the air admitted through the inlet 11 may be insufficient to effect complete combustion of the sulfur with the result that part of the sulfur 90 will be vaporized and carried into the flue 5 along with the sulfur dioxid formed. It has been found that sulfur vapor so carried and burned by the subsequent addition of air does not combine with the ore but is 95 maintained in a vapor form. The mixed sulfur dioxid and sulfur vapor entering the roast hearth near the discharge end of the furnace travels in the opposite direction to the travel of the ore, and air is admitted 100 to the ore hearth as required for the subsequent and successive combustion of the charge and for the completion of the roast. The heat of the ore bed is sufficient to keep the sulfur volatilized while the admission 105 of air to the ore hearth as required generates heat which is utilized for completing the roasting operation.

In supplying to a greater or less extent the extraneous heat necessary for a dead 110 roast by the combustion of sulfur, instead of heating the ore bed in part directly and in part indirectly by the combustion of separate charges of sulfur, a single operation may be effected by burning the sulfur in one 115 of the lower gas flues, either completely or incompletely, and turning the resulting gas while still in a highly heated condition into an ore hearth. Where the sulfur has been incompletely burned in the gas flue or flues, 120 its combustion can be completed by the introduction of air after the products of incomplete combustion have been introduced into the ore hearth. In this case, the heat will be partly supplied indirectly and partly 125 directly by the progressive combustion of the charge of sulfur first in the gas flue and then in the ore hearth.

The furnace of Fig. 2 is of a similar construction to that of Fig. 1, but instead of 130

having a separate small furnace at one side of the multiple hearth furnace, one or more sulfur containing pans or receptacles 13 are provided, together with suitable regulable air inlets 11<sup>a</sup>, so that the sulfur will be burned and the resulting heat utilized in the ore hearths. Gas flues 3<sup>a</sup> and 4<sup>a</sup> are provided, similar to the flues 3 and 4 of Fig. 1, so that the heat generated by the combustion of the sulfur can be supplemented, if necessary, by indirect heating in the usual manner. The flues 3<sup>a</sup> and 4<sup>a</sup> communicate through a suitable connecting flue 14 in the furnace wall.

15 The lower ore hearth 5<sup>a</sup> and the upper ore hearths 6<sup>a</sup>, are similar in construction to the corresponding hearths of Fig. 1, the lower hearths 5<sup>a</sup> and 6<sup>a</sup> alternating with the gas flues 3<sup>a</sup> and 4<sup>a</sup>. Suitably pivoted doors 20 or closures 12 are provided at the ends of the ore flues, for the introduction of rakes, and for the removal of the ore from the lower hearth 5<sup>a</sup>. The pan or receptacle 13 for the sulfur is arranged above the hearth 25 5<sup>a</sup>, at its discharge end, this receptacle 13 being suitably supported by the furnace wall. It is shown as projecting a short distance beyond the end wall of the furnace, but, in practice, it may project from the side wall 30 of the furnace, in a manner not shown, instead of from the end wall. Where a plurality of receptacles 13 are used, they can be similarly arranged at such places along the furnace, or at different levels, as may be 35 found desirable for supplying the additional heat necessary.

The operation of the furnace of Fig. 2 is similar to that of the furnace of Fig. 1. The sulfur is burned near the discharge end of 40 the lower ore hearth and the products of combustion, or the mixed sulfur dioxid and sulfur vapors, pass in the opposite direction to the ore along the ore hearth, any sulfur vapors being successively and subsequently 45 burned to give further increments of heat, and the ore bed being hot enough to keep the sulfur volatilized.

As a result of the combustion of sulfur in 50 the furnace, not only is heat supplied to the ore charge for assisting or completing the final stages of the roast, but the escaping gases are materially enriched in sulfur dioxid, so that the escaping gases are of increased value where they are desired for 55 subsequent conversion into sulfuric acid.

Having thus described my invention, what I claim is:

1. The method of roasting ores and of enriching the roaster gases in sulfur dioxid, 60 which comprises burning sulfur in heat interchanging relation with the ore bed and thereby supplying heat thereto for promoting the roasting operation, and combining the products of combustion of the sulfur with the roaster gases and thereby enriching

the roaster gases in sulfur dioxid; substantially as described.

2. The method of roasting ores and of enriching the roaster gases in sulfur dioxid, 70 which comprises burning sulfur in contact with the ore bed and applying the heat of the combustion directly to the ore bed to promote the roasting operation and also burning sulfur in heat interchanging relation with the ore bed but not in direct contact therewith, and combining the products of combustion of the sulfur with the roaster gases and thereby enriching the roaster gases in sulfur dioxid; substantially as described.

3. The method of roasting ores and of enriching the roaster gases in sulfur dioxid, 75 which comprises burning sulfur incompletely, in indirect heating relation to the ore bed and subsequently completing the combustion of the sulfur in direct contact with the ore bed, whereby heat for promoting the roasting operation is in part supplied directly and in part indirectly by the combustion of sulfur, and whereby the 80 roaster gases are enriched in sulfur dioxid by the addition thereto of the products of combustion of the sulfur; substantially as described.

4. The method of roasting ores and of enriching the roaster gases in sulfur dioxid, 85 which comprises burning sulfur in direct contact with the ore bed, and thereby applying heat directly to the ore and enriching the furnace gases in sulfur dioxid; sub- 90 stantially as described.

5. The method of roasting ores in a multiple hearth furnace and of enriching the roaster gases in sulfur dioxid, which comprises burning sulfur in direct contact with the ore in the lower levels of the furnace, 105 and thereby supplying heat directly to the ore body for completing the roasting operation, and enriching the furnace gases in sulfur dioxid; substantially as described.

6. The method of roasting ores in a multiple hearth furnace and of enriching the roaster gases in sulfur dioxid, which comprises burning sulfur with insufficient air for complete combustion, in direct contact 110 with the ore in the lower levels of the furnace, and subsequently introducing further amounts of air for completing the combustion of the sulfur in contact with the ore bed, thereby supplying heat to the ore for 115 completing the roasting operation and enriching the sulfur gases in sulfur dioxid; substantially as described.

7. The method of roasting ores in a multiple hearth furnace and of enriching the 120 roaster gases in sulfur dioxid, which comprises burning sulfur in the lower hearth of the furnace near the discharge end, and passing the products of combustion in the 125 direction opposite to the travel of the ore, 130

thereby supplying heat directly to the ore bed near its discharge from the furnace, and enriching the furnace gases in sulfur dioxid; substantially as described.

5 8. The method of roasting ores in a multiple hearth furnace and of enriching the roaster gases in sulfur dioxid, which comprises burning, in the lower levels of the furnace, sulfur with insufficient air to cause

complete combustion, and subsequently introducing further amounts of air for completing the combustion, thereby supplying heat directly to the ore bed in a progressive manner and enriching the furnace gases in sulfur dioxid; substantially as described. <sup>10</sup> <sup>15</sup>

In testimony whereof I affix my signature.

**ALBERT B. NEWMAN.**

Corrections in Letters Patent No. 1,280,283.

It is hereby certified that in Letters Patent No. 1,280,283, granted October 1, 1918, upon the application of Albert B. Newman, of Langlooth, Pennsylvania, for an improvement in "Processes of Roasting Ores," errors appear in the printed specification requiring correction as follows: Page 3, line 21, for the word "flues" read *hearths*; same page, line 70, claim 2, before the word "contact" insert the word *direct*; and that the said Letters Patent should be read with these corrections therein that the same may conform to the record of the case in the Patent Office.

Signed and sealed this 29th day of October, A. D., 1918.

[SEAL.]

R. F. WHITEHEAD,

*Acting Commissioner of Patents.*

Cl. 23—1.